

Patented Apr. 7, 1925.

1,532,427

# UNITED STATES PATENT OFFICE.

RICHARD METZGER, OF HEIDELBERG, GERMANY, ASSIGNOR TO BADISCHE ANILIN- & SODA-FABRIK, OF LUDWIGSHAFEN-ON-THE-RHINE, GERMANY, A CORPORATION OF GERMANY.

## TREATMENT OF CELLULOSE ESTERS FOR DYEING.

No Drawing.

Application filed October 18, 1924. Serial No. 744,494.

To all whom it may concern:

Be it known that I, RICHARD METZGER, citizen of the German Empire, residing at Heidelberg, Germany, have invented new and useful Improvements in the Treatment of Cellulose Esters for Dyeing, of which the following is a specification.

It is known that cellulose esters, especially cellulose acetate, have a limited capacity for taking up coloring matters. Various suggestions have already been made to remove this drawback, such as an addition of glycerol acetate or other organic acid esters of glycerol to the cellulose esters or to the dye-baths. Such compounds however have a dissolving effect on cellulose ester and are therefore liable to attack or destroy the fibres and articles made from them.

I have now discovered that the capacity of cellulose esters for taking up dyestuffs can be considerably increased without any injurious action by treating them with a bath containing a dissolved ester of a mineral oxygen acid, especially salts of acid esters of a mineral oxygen acid. Salts of acid esters of sulfuric or phosphoric or boric acid may be cited as examples. The said esters, or ester salts, may be used in a separate bath applied to the fibre, or article, preparatory to the dyeing or they may be added to the dyeing bath. The treatment may be done either at ordinary or elevated temperature. For example very good results are obtained when the fibre is put into an aqueous solution containing a compound of the aforesaid character and allowing it to stand for quite a while at ordinary temperature.

The following examples serve to further explain the nature of the invention but the invention is not restricted to these examples.

### Example 1.

10 kilogrammes of cellulose acetate silk are treated, for about 10 minutes, at between about 50 degrees and 60 degrees centigrade, with 300 litres of a 50 per cent, by weight, solution of potassium ethyl sulfate with a little acetic acid, the silk so treated is then wrung out, stretched and dyed, without previous rinsing, at between 40 degrees and 70 degrees centigrade with 1 per cent of

diamond green B in a bath slightly acidulated with acetic acid.

55

### Example 2.

10 kilogrammes of cellulose acetate silk are dyed, while gradually raising the temperature from 40 degrees up to 70 degrees centigrade, in a bath containing 200 litres of water, 100 grammes of auramine II, a little acetic acid and 6 kilogrammes of a 30 per cent aqueous solution of sodium dicresyl phosphate.

60

65

### Example 3.

1 kilogramme of cellulose acetate silk is handled for about 10 minutes in 30 litres of a 5 or 6 per cent solution of sodium dicresyl phosphate in water. This preliminary treatment may take place either at ordinary or elevated temperature. The silk is then wrung out, stretched and dyed with 0.8 per cent of methyl violet 2B extra at from 40 degrees to 70 degrees centigrade with or without an addition of purified waste sulfite cellulose liquor. The fibre prepared as before described may also be dyed with 1 per cent of azoflavine RS in a bath weakly acidulated with acetic acid.

70

75

80

### Example 4.

1 kilogramme of cellulose acetate silk is treated, at between 40 degrees and 50 degrees centigrade with 30 litres of a 10 per cent solution of sodium dicresyl phosphate, wrung out and dyed with 10 per cent indanthrene blue GCD paste with or without an addition of a protective colloid in a dyebath containing, in each litre, 3 cubic centimetres of caustic soda lye, of 40 degrees Baumé, 2 grammes of sodium hydro-sulfite concentrated powder and 10 grammes of calcined Glauber's salt at a temperature of 40 degrees centigrade. Then soap as usual.

85

90

95

What I claim is:

1. The process of treating cellulose esters for dyeing which consists in treating the cellulose esters in a bath containing an ester of a mineral oxygen acid.
2. The process of treating cellulose acetate for dyeing which consists in treating the cellulose ester in a bath containing a salt of an acide ester of a mineral oxygen acid.

100

105

3. The process of treating cellulose acetate for dyeing which consists in treating the fibre in a bath containing a salt of an acid ester of phosphoric acid.
4. The process of treating cellulose acetate fibre for dyeing which consists in treating the fibre in a bath containing a salt of an acid ester of phosphoric acid and subsequently dyeing the fibre so treated in a dye-stuff solution.
5. The process of treating cellulose acetate fibre for dyeing which consists in treating the fibre in a bath containing a salt of an acid ester of phosphoric acid and subsequently dyeing the fibre so treated in a dye-stuff solution.

10

In testimony whereof I have hereunto set my hand.

RICHARD METZGER.

Attest:

A. H. GERNERT,  
JANE GINSTI.